

1

3,232,695

**PROCESS FOR DYEING MATERIALS BASED ON POLYAMIDES AND COMPOSITIONS THEREFOR**

Jean-Baptiste Robin, Lyon, and Jean Etienne Rappin, Collonges-au-Mont-d'Or, France, assignors to Societe Rhodiaceta, Paris, France, a corporation of France  
 No Drawing. Filed Nov. 21, 1962, Ser. No. 239,356  
 Claims priority, application France, Nov. 22, 1961,  
 879,739

7 Claims. (Cl. 8—55)

This application is a continuation-in-part of application Serial No. 222,653, filed September 19, 1962, and now abandoned. As such, this application is entitled to the priority date of November 22, 1961, under U.S.C. 119 for French application Serial No. 879,739.

The present invention relates to a new process for colouring materials based on polyamides, by means of which it is possible to obtain very level, intense shades of good fastness without deterioration of the material and to new compositions for carrying out the new process.

It is known to dye textile articles consisting of polyamides with dyes of the acid type by adding to the dyeing bath products having anionic character, as also products having a slightly cationic character. Uniform dyes free from streaks are thus obtained.

It is also known to treat textile articles of polyamides in aqueous medium at temperatures above 100° C. in the presence of a reducing product containing sulphur. It is possible by this method to avoid yellowing of polyamides by aqueous treatment at high temperature and thus dulling of the colours and degradation of the dyed material.

There has now been discovered, and this forms the subject of the present invention, a new process for dyeing polyamide materials by means of which it is possible to obtain even better and hitherto unachieved results.

The process according to the invention consists in dyeing materials based on polyamides, at a temperature of at least 90° C., in a bath having a pH between 3 and 5, in the simultaneous presence of:

(a) An anionic levelling agent and preferably a compound of the formula:  $R(A)_nR'$ , where R and R' each represents a sulphonated naphthalene or benzene nucleus which may be the same or different, A represents one of the radicals  $CH_2$ ,  $SO_2$  or  $NH$ , and n is an integer between 0 and 4 inclusive;

(b) A weakly cationic complexing agent and particularly polyvinyl pyrrolidone or a product of condensation of ethylene oxide with a long-chain fatty amine or an aromatic amine, and

(c) Thiourea or one of its N-alkylated derivatives, such as N-monomethylthiourea.

Compositions comprising the above three ingredients are novel and form part of the present invention. They may be alone or in mixtures with solid or liquid inert products in solution, emulsion, or dispersion but are preferably in the form of an aqueous solution.

Particularly suitable anionic levelling agents are the sodium or other alkali metal salts of  $\alpha,\alpha'$ -dinaphthyl- $\beta,\beta'$ -disulphonic acid, or of  $\alpha,\alpha'$ -dinaphthylmethane- $\beta,\beta'$ -disulphonic acid, while the substances sold under trade names Neovadine AN and Neolisal, and the condensation products of ethylene oxide and laurylamine, oleylamine and stearylamine are particularly useful cationic complexing agents.

Applicants have discovered that the combination of all the dyeing conditions hereinbefore enumerated leads to results which have hitherto never been obtained.

The invention makes it possible to produce shades which are brighter and faster to washing than when dyeing is effected by previously known methods.

Moreover, it is possible by means of the invention to

2

avoid streakiness more readily than when dyeing with one of the hitherto known methods, because the presence of thiourea or one of its alkyl derivatives during the dyeing simultaneously prevents any oxidation of the polymers to be dyed and, therefore, any degradation of the dyed material and, in addition, prevents inequalities in dyeing which result in the formation of streaks.

This is true in the case of simple acid dyes and in the case of metalliferous acid dyes, and even in the case of reactive dyes of acid character, which is rather remarkable.

Moreover, the results obtained by employing the process according to the invention are achieved without difficulty, the application of the said process being simple and easy.

The dyeing with simple acid or 1:1 or 2:1 metalliferous acid dyes may be carried out in a single step in the acid medium without first applying an alkaline pretreatment step. It is, however, necessary for all three types of adjuvants hereinbefore enumerated to be present in the dyeing medium. The operation may be carried out in a bath either between 90° C. and 100° C. at atmospheric pressure or under pressure between 100° C. and a temperature just below that corresponding to the commencement of the deterioration either of the material to be dyed or of the dyestuff, which temperature may range up to 150° C. or more. Dyeing under pressure in an autoclave substantially improves the fastness and the levelness of the colouration obtained. Dyeing is carried out in an acid medium at a pH between 3 and 5, which is obtained by the addition of a mineral acid or of an organic acid, for example acetic acid or formic acid.

On the other hand, when applying the various reactive dyestuffs of acid character an alkaline treatment, preferably at a relatively low temperature, is advantageous. In the case of the dyeing of textile materials, for example, this pretreatment is carried out at a temperature between the ambient temperature, for example 20° C. and 50° C., at a pH adjusted between 10 and 12. The second step or dyeing process may be carried out in the same bath or in a second bath, under the conditions specified in the preceding paragraph.

The use of a reducing agent containing sulphur in the treatment of textile materials consisting of polyamides is known but applicants have discovered that when thiourea or an alkyl derivative thereof is employed in traces in the dyeing medium, together with the anionic levelling agent and the cationic agent, it behaves as an anti-oxidising catalyst. It is this catalysing function which has made it possible to obtain a quality of dyeing which could not have been foreseen from the known properties of certain anionic agents and certain cationic agents.

In this connection it is to be noted that the quantities of thiourea, of anionic agent and of cationic agent to be employed in the dyeing medium vary substantially as an inverse function of the quantity of dyestuff. For example, in the case of a dyebath for textile materials the following quantities of thiourea, expressed in percentage of material treated, are suitable:

|    | Dyestuff, percent: | Thiourea, percent |
|----|--------------------|-------------------|
| 60 | >2                 | 0.02              |
|    | 1 to 2             | 0.03              |
|    | 0.5 to 1           | 0.04              |
| 65 | <0.5               | 0.05              |

The small quantities of thiourea necessary demonstrate that its action is essentially catalytic.

In addition to the aforesaid advantages, it is to be noted that the present process, in contradistinction to conventional methods for improving the levelness of dyeing with acid or metalliferous dyes on polyamide materials, does

not in any way reduce the yield of the dyes on the materials, but in the majority of cases the yield is even substantially improved, so that it is possible to reduce the usual dyeing times.

Finally, the presence of thiourea or an alkyl derivative thereof does not give rise to change in shade as is the case with other active antioxidising or reducing agents.

The process according to the invention produces a true protective effect on materials based on polyamides and prevents or retards degradation thereof by oxidation. In an aqueous bath at high temperature, very small quantities of oxygen are sufficient to produce a considerable modification of these materials. In practice, it is very difficult to eliminate air completely from the material to be dyed and from the dyeing medium, especially in the case of textile materials, and it has hitherto frequently happened that, for example, in the course of the dyeing of textured yarns, occluded air bubbles cause breakages in winding or weak points in made-up materials, and in addition, produce differences in shades on the yarns. These defects are obviated by the use of the process according to the present invention.

The invention is illustrated by the following examples in each of which thiourea itself is used for convenience. It may be replaced with equally good results by an alkyl derivative such as N-monomethylthiourea.

#### Example I

A dyebath is prepared containing, per 1500 litres of liquor, 750 g. of trisodium phosphate and 500 g. of the 30 dyestuff having the formula:



100 kg. of fabric consisting of polyamide 66 continuous filament yarn of 4.4 tex. (40 denier) 13 filaments, 200 Z turns per metre are treated in the bath for 10 minutes at 40° C. There are then added 0.75 l. of glacial acetic acid, 400 g. of formic acid (80% by weight), 2.5 kg. of the condensation product of ethylene oxide and laurylamine, 2.5 kg. of sodium  $\alpha,\alpha'$ -dinaphthylmethane- $\beta,\beta'$ -disulphonate and 50 g. of thiourea. Dyeing is carried out for 1 hour at 100° C., whereafter the product is rinsed in a 1000-litre bath containing 500 g. of the condensation product of a fatty alcohol and ethylene oxide, commercially known under the name Sunaptol O. After washing and drying, the fabric has a fine pale-yellow colouration which is fast to washing and completely level. The fabric has undergone no degradation.

#### Example II

The procedure of Example I is followed, using a dye-stuff of the formula:



and the following quantities:

|                                                                          |        |       |
|--------------------------------------------------------------------------|--------|-------|
| Bath                                                                     | litres | 1500  |
| Dye                                                                      | kg     | 3     |
| Trisodium phosphate                                                      | kg     | 0.750 |
| Thiourea                                                                 | g      | 30    |
| Sodium $\alpha,\alpha'$ -dinaphthylmethane- $\beta,\beta'$ -disulphonate | kg     | 1.5   |
| Product sold under trade name "Neolisal"                                 | kg     | 1.5   |
| Fabric                                                                   | kg     | 100   |

In the second phase of the dyeing, the bath is neutralised with 750 g. of glacial acetic acid, and acidified with 400 g. of formic acid (80%).

The dyed fabric has a very fast red colouration of excellent levelness, while having retained its initial mechanical properties.

#### Example III

20 The procedure of Example II is followed, by using a dyestuff of the formula:



A blue colouration is obtained of remarkable fastness. The fabric exhibits no streaky or stripy effects.

#### Example IV

100 kg. of a fabric consisting of polyamide 6 continuous filament yarns of 7.7 tex. (70 denier) 23 filaments 200 Z turns per metre are dyed in 1000 l. of water containing 1 kg. of a dyestuff of the formula:



2 kg. of sodium  $\alpha,\alpha'$ -dinaphthylmethane- $\beta,\beta'$ -disulphonate

2 kg. of the product commercially known under the trade name Neovadine AN,

40 g. of thiourea,

The pH of the bath is adjusted to 3 by means of acetic acid.

The fabric is dyed for 1 hour at 120° C. and rinsed and dried.

The fabric has a very bright blue colour of excellent fastness to light and even to very vigorous washing, and is completely level, while having retained its good mechanical properties.

#### Example V

Piece goods made from stable fibre yarns, each 77 tex./3 x 270 Z/160 S, of polyamide 11 is dyed under 75 the same conditions as in Example IV, but replacing the

dyestuff there employed by a dyestuff having the following formula:



The fastness properties of the dyeing obtained are as good as those in Example IV.

The dyeing is a fine deep fast black having no streaks. When polyamide materials are dyed with the same dyes as in the above examples, but omitting one or more of the conditions characteristic of the invention, dyeings are obtained whose shades are distinctly less bright and considerably less level.

*Example VI*

100 kg. of a fabric made of polyamide 66 continuous filament yarn is introduced into a dye bath containing 1000 l. of water to which has been added 2 kg. of Acid Red 211 (Colour Index Second Edition 1956, Part I, vol. I, page 1180), and 2.5 l. of an aqueous solution containing (a) 392 g. per litre of the condensation product of laurylamine with ethylene oxide, (b) 392 g. per litre of sodium dinaphthyl methane disulphonate and (c) 16 g. per litre of thiourea.

The pH of the bath is adjusted to 3.5 by means of glacial acetic acid. Dyeing is carried out for one hour at 130° C. whereupon the fabric is rinsed and dried. The resulting fabric is dyed in a perfectly level shade of red and retains its initial mechanical properties.

We claim:

1. Process for dyeing synthetic polyamide materials, comprising dyeing the materials in a dyebath at a temperature of at least 90° C., the dyebath having a pH of between 3 and 5 and containing

(a) an anionic leveling agent having the formula  $R(A)_nR'$ , wherein R and R' each represent a sulphonated aromatic nucleus selected from the group consisting of benzene and naphthalene nuclei, A is a divalent radical selected from the group consisting of  $-\text{CH}_2-$ ,  $-\text{SO}_2-$  and  $-\text{NH}-$ , and n is an integer between 0 and 4 inclusive,

(b) a weekly cationic complexing agent selected from the group consisting of polyvinyl pyrrolidone, condensation products of ethylene oxide with long chain fatty amines and condensation products of ethylene oxide with aromatic amines,

(c) a catalytic amount of a substance selected from the group consisting of thiourea and N-alkylated thioureas

(d) an anionic dyestuff.

2. Process for dyeing synthetic polyamide materials comprising first pretreating the materials in an alkaline bath of pH between 10 and 12 at a temperature of 50° C.

at most and then dyeing the materials in a dyebath at a temperature of at least 90° C., the dyebath having a pH of between 3 and 5 and containing

(a) an anionic leveling agent having the formula  $R(A)_nR'$ , wherein R and R' each represent a sulphonated aromatic nucleus selected from the group consisting of benzene and naphthalene nuclei, A is a divalent radical selected from the group consisting of  $-\text{CH}_2-$ ,  $-\text{SO}_2-$  and  $-\text{NH}-$ , and n is an integer between 0 and 4 inclusive,

(b) a weekly cationic complexing agent selected from the group consisting of polyvinyl pyrrolidone, condensation products of ethylene oxide with long chain fatty amines and condensation products of ethylene oxide with aromatic amines,

(c) a catalytic amount of a substance selected from the group consisting of thiourea and N-alkylated thioureas

(d) an anionic dyestuff.

3. Process for dyeing synthetic polyamide materials, comprising dyeing them at a temperature above 90° C. in a dyebath having a pH between 3 and 5 and containing an acid dyestuff, an alkali metal salt of  $\alpha,\alpha'$ -dinaphthylmethane- $\beta,\beta'$ -disulphonic acid, thiourea and condensation product of ethylene oxide and an amide selected from the group consisting of laurylamine, oleylamine and stearylamine.

4. Process according to claim 3, wherein dyeing is preceded by a treatment of the material in an alkaline bath of pH between 10 and 12 at a temperature up to 50° C.

5. Process according to claim 6, wherein the anionic dyestuff is present both in the alkaline pretreatment bath and in the acid dyebath.

6. Process for dyeing synthetic polyamide materials, comprising first treating the materials in an alkaline bath at pH between 10 and 12 to a temperature up to 50° C. and thereafter adding to the bath

(a) an anionic leveling agent having the formula  $R(A)_nR'$ , wherein R and R' each represent a sulphonated aromatic nucleus selected from the group consisting of benzene and naphthalene nuclei, A is a divalent radical selected from the group consisting of  $-\text{CH}_2-$ ,  $-\text{SO}_2-$  and  $-\text{NH}-$ , and n is an integer between 0 and 4 inclusive,

(b) a weekly cationic complexing agent selected from the group consisting of polyvinyl pyrrolidone, condensation products of ethylene oxide with long chain fatty amines and condensation products of ethylene oxide with aromatic amines,

(c) a catalytic amount of a substance selected from the group consisting of thiourea and N-alkylated thioureas,

(d) an anionic dyestuff.

7. Composition of matter for use in dyeing synthetic polyamide articles in level shades with anionic dyestuffs, comprising in combination,

(a) an anionic leveling agent having the formula  $R(A)_nR'$ , wherein R and R' each represent a sulphonated aromatic nucleus selected from the group consisting of benzene and naphthalene nuclei, A is a divalent radical selected from the group consisting of  $-\text{CH}_2-$ ,  $-\text{SO}_2-$  and  $-\text{NH}-$ , and n is an integer between 0 and 4 inclusive,

(b) a weekly cationic complexing agent selected from the group consisting of polyvinyl pyrrolidone, condensation products of ethylene oxide with long chain fatty amines and condensation products of ethylene oxide with aromatic amines,

(c) a catalytic amount of a substance selected from the group consisting of thiourea and N-alkylated thioureas.

**References Cited by the Examiner**  
**UNITED STATES PATENTS**

|           |         |              |        |    |
|-----------|---------|--------------|--------|----|
| 1,867,022 | 7/1932  | Munz         | 8-84 X |    |
| 1,987,583 | 1/1935  | Berthold     | 8-85 X | 5  |
| 2,254,965 | 9/1941  | Kling        | 8-84 X |    |
| 2,404,769 | 7/1946  | Amick        | 8-85   |    |
| 2,623,806 | 12/1952 | Fuchs        | 8-84 X |    |
| 2,726,133 | 12/1955 | Helfenberger | 8-54   |    |
| 2,888,313 | 5/1959  | Mautner      | 8-85 X | 10 |
| 2,900,218 | 8/1959  | Gray         | 8-54   |    |
| 2,903,325 | 9/1959  | Geigy        | 8-85 X |    |
| 2,905,713 | 9/1959  | Schmidt      | 8-85 X |    |

|           |        |         |            |
|-----------|--------|---------|------------|
| 2,952,506 | 9/1960 | Dellis. |            |
| 2,971,813 | 2/1961 | Moran   | ----- 8-85 |

**OTHER REFERENCES**

Diserens Chemical Technology of Dyeing and Painting, vol. 2, pages 311-325, 338-341, pub. by Reinhold Publishing Corp., 1951.

Holmes, "American Dyestuff Reporter," pages 702-704.

McGrew, "American Dyestuff Reporter," page 136, Feb. 19, 1951.

NORMAN G. TORCHIN, *Primary Examiner*.

ABRAHAM H. WINKELSTEIN, *Examiner*.